

Patented Nov. 15, 1927.

1,648,947

# UNITED STATES PATENT OFFICE.

ERNEST H. JACOBS, OF CHICAGO, ILLINOIS, ASSIGNOR TO ELECTRICAL ENGINEERS EQUIPMENT COMPANY, OF CHICAGO, ILLINOIS, A CORPORATION OF ILLINOIS.

## ART OF REFINING COPPER.

No Drawing.

Application filed March 26, 1923. Serial No. 627,566.

My invention relates to the art of casting pure copper.

In the electrical industry it is highly desirable that pure copper of high conductivity 5 be employed particularly in connection with heavy current conducting apparatus where great amounts of cast copper are employed.

The desirability for a low resistance is obvious where high current values prevail 10 because the  $I^2 R$  losses run into large quantities.

Whereas the prior art has known it to be desirable to reduce the resistance, or in other terms increase the conductivity, of such 15 metal as is used in the transmission of heavy electric current, there has not been on the market any commercially successful method of casting copper which would bring the conductivity any higher than from 40 to 20 50% of that of rolled copper.

Where the conductivity is low there is not only the loss in power due to heating, but also a tendency to increase the weight of 25 the castings in an attempt to gain greater conductivity with a consequently greater investment in copper and consequently greater fixed interest charge for the station. According to my invention it is possible to produce copper which is substantially chemically 30 pure, which has a beautiful copper color, great density and high conductivity of the order of from 80 to 90% of that of rolled copper and in some cases higher than 90%.

In order to secure copper of this character, I employ a reducing agent or what I term herein a flux or alloy for purifying the molten copper just before it is cast into the 35 mold.

This reducing agent or alloy is produced 40 as follows:

First I take in the proportion of 10 pounds of phosphor copper and melt the same in a crucible under a thin blanket or covering of 45 charcoal. This is an alloy or metal which is well known and which I buy in the open market. The material in the crucible is still covered with charcoal and is thoroughly melted. Then I add in the proportion of 50 one pound of copper sulphate. After these ingredients are brought to the liquid state I then add in the proportion of one-half pound of fluorspar and after the above ingredients are brought to the liquid state by heating 55 to melt the same, I add the final ingredient

of and in the proportion of one-half pound of borax. This is then all finally brought to molten condition, the top of the crucible still being covered by a thin covering or blanket of charcoal. The above alloy or flux is then 60 cast into rods or thin strips in a suitable open or closed mold.

In the process of casting the copper I employ the flux or alloy as above prepared according to the following procedure.

The copper for producing castings which should be as clear as possible is melted in a crucible kept covered by a layer or blanket of charcoal. It is advisable to melt the copper in small crucibles.

Then, just as the crucibles are taken from the furnace prior to pouring I add the above flux or alloy in substantially the proportion of 9 ounces of flux or alloy to 200 pounds of molten copper. The above ratio is in approximately 70 the proportion of one half ounce of the alloy for each 10 pounds of molten copper.

In making the molds it is desirable to lay the castings flatwise, that is to say, with 80 as little depth in the casting as possible, and to employ a relatively large and free sprue in proportion to the gate so that by gravity the lighter ingredients may separate into the top of the sprue and the denser copper 85 remain at the bottom and form the casting.

Castings made according to the above procedure have a beautiful copper color, have a very high conductivity of the order of 80 to 90% of that of rolled copper of a conductivity of 100% Matthieson standard and are substantially chemically pure. It appears that the ingredients which make up the flux or alloy disappear from the main body of the copper and consequently they 90 do not appear in a chemical analysis of the castings.

I do not intend to be limited to the precise formula and method of procedure above stated, because in some instances where the 100 impurities of the copper supply the necessary re-agents or render them unnecessary they may be reduced or dispensed with. However, I have conducted considerable experimentation and have tested various deviations from the above formula but find them to be less satisfactory than the process and formula above outlined. This process and formula secures, so far as I can find, uniform results and the resulting castings are 105 110

as I find by a period of testing them in actual use, not subject to deterioration through ageing or weathering.

I claim:

- 5 1. The process of casting copper which comprises melting under a blanket of reducing material such as charcoal, a batch of copper, and adding to the melted copper a conditioning or purifying alloy or flux 10 in approximately the proportion of 9 ounces of said alloy or flux to 200 pounds of copper, said flux being added just prior to pouring the copper, comprising substantially the following constituents, namely, copper 10 15 pounds, phosphor copper three pounds, copper sulphate one pound, fluorspar one half pound, and borax one half pound.

2. The process of making a flux for casting copper which comprises melting under 20 a charcoal blanket, 10 pounds of copper, adding three pounds of phosphor copper, bringing the resulting material to a liquid state by heating, then adding one pound of

copper sulphate and again bringing the resulting material to a liquid state by heating, 25 then adding one half pound of fluorspar and again bringing the resulting material to a liquid state by heating and finally adding a half pound of borax and bringing the resulting material to a liquid state by heating. 30 3. A reducing agent or flux for molten copper consisting of the following ingredients in substantially the following proportions:

|                          | Per cent. | 35               |
|--------------------------|-----------|------------------|
| 10 pounds copper         |           | 66 $\frac{2}{3}$ |
| 3 pounds phosphor copper |           | 20               |
| 1 pound copper sulphate  |           | 6 $\frac{2}{3}$  |
| 1/2 pound fluorspar      |           | 3 $\frac{1}{3}$  |
| 1/2 pound borax          |           | 3 $\frac{1}{3}$  |
| 15 pounds                |           | 100              |

In witness whereof, I hereunto subscribe my name this 24 day of March, 1923.

ERNEST H. JACOBS.